

## UNITED STATES PATENT OFFICE

1,920,262

## ALUMINUM ALLOY

Louis W. Kempf and Walter A. Dean, Cleveland,  
Ohio, assignors to Aluminum Company of  
America, Pittsburgh, Pa., a Corporation of  
Pennsylvania

No Drawing. Application July 23, 1932  
Serial No. 624,345

2 Claims. (Cl. 75—1.)

This invention relates to aluminum base alloys characterized, at elevated temperatures, by high physical properties. Such alloys are used, for instance, in the manufacture of pistons or cylinder heads for internal combustion engines or in other adaptations where temperatures of use frequently considerably exceed room temperatures.

Alloys of the general nature herein described have already been disclosed in the copending application of R. S. Archer and L. W. Kempf, Serial No. 403,353, filed October 29, 1929, and in the copending application of W. A. Dean, Serial No. 552,557, filed July 22, 1931. These copending applications relate to aluminum base alloys containing copper, silicon, and nickel, the copper not exceeding 8 per cent. In application Serial No. 403,353 aforementioned, there is disclosed an alloy exhibiting said high temperature properties and sufficient strength at room temperature to fully serve its purpose. In application Serial No. 552,557 aforementioned, there is disclosed an alloy which, by reason of a certain nickel content, has a high strength in the cast condition, a considerably refined crystalline structure, and an increased ductility, these properties being obtained without material impairment of the properties which characterize the alloys disclosed in the earlier application Serial No. 403,353.

We have discovered that it is possible, by a modification of the earlier known alloys of this type, to simultaneously preserve the advances made in the latest exemplifications of so-called high temperature alloys and at the same time effect further improvement in the properties of the alloy at elevated temperatures, namely, in the neighborhood of 400° Fahrenheit to 600° Fahrenheit. This we have accomplished by providing an aluminum base alloy having a nickel content of about 2 per cent to about 6 per cent by weight, a silicon content of about 5 per cent to about 12 per cent by weight, and a copper content above 8 per cent, the copper content usually being about 9 per cent to about 14 per cent by weight. The balance of the alloy may be aluminum in any of the grades which are available commercially. The alloy may likewise contain from about 0.01 per cent to about 1 per cent of a high melting point metal, such as titanium, molybdenum, tungsten, manganese, chromium, or iron. More than one of these high melting point metals may be used in combination, provided their total amount does not exceed about 1 per cent of the whole. In alloys of the above

composition, we have secured very favorable physical properties at elevated temperatures, including higher hardness and tensile strength and, in addition, a relatively high impact resistance at all temperatures and better tensile properties at room temperatures.

In order to describe some of the advantages of our alloys, the following is a comparison between alloy A, which is the preferred alloy made in accordance with our invention, and alloys B and C, which represent alloys known prior to our invention and disclosed in the aforesaid copending applications. The compositions of alloys A, B, and C are set forth in the following table:

Table I

| Alloy | Cu<br>percent<br>by<br>weight | Si<br>percent<br>by<br>weight | Ni<br>percent<br>by<br>weight | Commer-<br>cial Al |
|-------|-------------------------------|-------------------------------|-------------------------------|--------------------|
| A     | 12                            | 7                             | 4                             | Balance.           |
| B     | 7                             | 7                             | 7                             | Balance.           |
| C     | 7                             | 7                             | 4                             | Balance.           |

Since experience has demonstrated that for properly evaluating two or more alloys with reference to their behavior at elevated temperatures, the alloys should be tested under substantially identical conditions, factors such as the length of time at temperature before testing, initial thermal treatments, rate at which the load is applied in tensile testing, etc., were maintained as nearly equal as possible in the tests about to be described.

Alloy A in the sand cast condition had a tensile strength at room temperature of 25,300 pounds per square inch. At a temperature of 400° Fahrenheit, the alloy had a tensile strength of 24,800 pounds per square inch, and at 600° Fahrenheit the alloy had a tensile strength of 18,000 pounds per square inch.

A sand casting made of alloy B had a tensile strength of 19,000 pounds per square inch at room temperature. At 400° Fahrenheit, its tensile strength was 17,000 pounds per square inch, and at 600° Fahrenheit its tensile strength was 12,700 pounds per square inch.

Alloy C, sand cast, had a tensile strength at room temperature of 27,000 pounds per square inch. At 400° Fahrenheit, the tensile strength of alloy C was about 24,000 pounds per square inch, and at 600° Fahrenheit the tensile strength of alloy C was about 15,500 pounds per square inch.

Upon comparison of the properties of A, B, and C, it will be noted that alloy A lost only

about 500 pounds per square inch in tensile strength when the temperature was raised from room temperature to 400° Fahrenheit, while alloy B, under the same conditions, lost 2,000 pounds per square inch in tensile strength. As the temperature was raised to 600° Fahrenheit, it will be noted that the tensile strength of alloy A was only 1,000 pounds per square inch less than the tensile strength of alloy B at room temperature, and that the tensile strength of alloy A at 600° Fahrenheit exceeded the tensile strength of alloy C by about 2,500 pounds per square inch, alloy C having lost in tensile strength about 12,000 pounds per square inch while alloy A lost only about 7,000 pounds per square inch.

Another interesting comparison which illustrates the advantageous properties of the alloys which are the subject of this invention are the comparative impact resistance values in a standard impact testing machine both at room temperature and at 600° Fahrenheit. At room temperature alloy A has an impact resistance of 64.5 foot pounds per square inch and alloy B has an impact resistance of 47.5 foot pounds per square inch. At 600° Fahrenheit alloy A has an impact resistance of 66.5 foot pounds per square inch and

alloy B has an impact resistance of 46.0 foot pounds per square inch.

The alloys which are the subject of the present invention may be heat-treated for the purpose of improving their tensile and hardness properties or they may be otherwise thermally treated for the purpose of removing strains or stabilizing volume changes. For such purposes, the heat-treatment and other thermal processes well known to those skilled in the art may be used.

What we claim is:

1. An alloy consisting of about 12 per cent by weight of copper, about 7 per cent by weight of silicon, and about 4 per cent by weight of nickel, the balance being substantially aluminum.

2. An alloy consisting of from 9 to about 14 per cent by weight of copper, from about 5 to about 12 per cent by weight of silicon, and from about 2 to about 6 per cent by weight of nickel, the balance being substantially aluminum, said alloy being characterized by an internal structure relatively highly resistant to deterioration of properties under the influence of elevated temperatures.

LOUIS W. KEMPF. 100  
WALTER A. DEAN.

30

105

35

110

40

115

45

120

50

125

55

130

60

135

65

140

70

145

75

150